

Jan. 1, 1957

J. H. MOORE

2,776,204

PRODUCTION OF METALS

Filed Jan. 22, 1952

2 Sheets-Sheet 1



FIG. 1



FIG. 2

INVENTOR.  
JAMES H. MOORE

BY

Oliver W. Hayes

ATTORNEY

Jan. 1, 1957

J. H. MOORE

2,776,204

PRODUCTION OF METALS

Filed Jan. 22, 1952

2 Sheets-Sheet 2



1

2,776,204

## PRODUCTION OF METALS

James H. Moore, Swampscott, Mass., assignor to National Research Corporation, Cambridge, Mass., a corporation of Massachusetts

Application January 22, 1952, Serial No. 267,670

8 Claims. (Cl. 75—49)

This invention relates to the production of metals and more particularly to the production of high purity iron and iron alloys.

The production of iron and certain iron alloys of very high purity has hitherto been limited in scale because of the difficulty of eliminating contamination by the atmospheric gases. It has long been recognized that nitrogen and hydrogen may be readily removed from iron by heating the iron in a high vacuum. However, the problem of removing oxygen is considerably more involved. The addition of deoxidizing elements, such as aluminum and silicon, can reduce the oxygen in solution, but such additions may be prohibitive because of the amount of the deoxidizing element required to be left in solution at equilibrium to assure the necessary degree of deoxidation. Thus, for example, the amounts of aluminum, carbon, or silicon in solution in iron, in equilibrium with an oxygen content of 0.005%, are approximately 0.15%, 0.55%, 1.5%, respectively. In the case of one of the deoxidants (i. e., carbon) it has been previously proposed that a low oxygen content could be obtained in iron and iron-silicon alloys by the use of vacuum-melting techniques.

In this proposed prior art method an accurate oxygen and carbon analysis is first made of the charge and then either one or the other of these elements is added to stoichiometrically balance the analysis for the reaction of carbon and oxygen to form carbon monoxide. The charge is then melted in a vacuum for a sufficient time for the pressure to reach a low value after the initial pressure increase which is due to the carbon monoxide formation resulting from the reaction between oxygen and carbon in the melt. This low value has been said to be preferably 10 microns (0.01 mm.) or less, this low pressure being obtained in from one to twelve hours. This technique is satisfactory if extremely accurate analyses of the oxygen and carbon contents of the iron are possible, and also if no contamination of the molten iron is introduced by reaction between the molten iron and the crucible. However, it is extremely difficult to obtain an accurate carbon and oxygen analysis for the charge in those cases where it is difficult to obtain a representative sample, such as when the pieces of iron vary in shape and degree of oxidation, for example when electrolytic flake is used as a source of the iron to be purified. In large charges where several pieces of iron are being purified in a single melt, an absolutely representative sample is almost impossible to obtain.

While there are several types of crucible materials which do not have an appreciable reaction with molten iron under vacuum at temperatures of the order of 1600° C. and above, these crucible materials, such as zirconia or beryllia, are extremely expensive and cannot be employed for producing pure iron in commercial quantities. The normally employed commercial refractories, such as alumina, silica, zircon and magnesia, are unsatisfactory from the standpoint of contamination when utilized with molten iron in a vacuum furnace unless they are employed in accordance with the present invention.

2

Of the above mentioned commercially available refractories, magnesia is probably the most interesting. At steel-making temperatures, and at atmospheric pressure, it is very stable and gives rise to no contamination in the melting of iron. Furthermore, its resistance to thermal shock is good. However, when one considers the stability of magnesia at low pressures, it is evident from thermochemical calculations that, at equilibrium, the degree of contamination by oxygen will be considerable by reason of the volatility of magnesium which drives the reduction of MgO by molten iron. Thus, it would appear that it is impossible to hold iron in magnesia at low pressures for extended periods of time without contamination in excess of 0.1% oxygen because of the unfavorable equilibrium. This theoretical prediction has been verified experimentally. However, the present invention permits the use of such crucibles to obtain high purity iron.

Accordingly, a principle object of the present invention is to provide a method for producing high purity iron and iron alloys which eliminates the need for crucible material which is expensive and scarce.

Another object of the invention is to provide a process of the above type which employs a crucible material having a metallic constituent which is too volatile to be retained in the iron bath.

Still another object of the invention is to provide such a process which employs a dynamic purification to prevent oxygen contamination of the molten iron despite an unfavorable equilibrium between the molten iron and the material of the crucible.

Still another object of the invention is to provide such a process which obviates the necessity for accurate carbon and oxygen analyses of the charge prior to melting thereof.

Still another object of the invention is to provide new and improved apparatus for practicing the improved processes of the invention.

Still another object is to provide new iron alloys having improved fatigue strength.

Other objects of the invention will in part be obvious and will in part appear hereinafter.

The invention accordingly comprises the product possessing the features, properties and the relation of components; the process involving the several steps and the relation and the order of one or more of such steps with respect to each of the others; and the apparatus possessing the construction, combination of elements and arrangement of parts which are exemplified in the following detailed disclosure, and the scope of the application of which will be indicated in the claims.

For a fuller understanding of the nature and objects of the invention, reference should be had to the following detailed description taken in connection with the accompanying drawings wherein:

Fig. 1 is a graph showing oxygen, carbon, nitrogen and hydrogen content as a function of time during vacuum refining of iron;

Fig. 2 is a graph showing oxygen content as a function of carbon monoxide evolution rate;

Fig. 3 is a graph showing oxygen content as a function of pressure for a vacuum system whose time of pump-down is varied; and

Fig. 4 is a schematic, diagrammatic illustration of one preferred measuring and control system embodying the present invention.

In the present invention high purity iron having less than about 0.015% oxygen is obtained by a process which involves the use of relatively inexpensive crucibles which predominate in magnesia. In practicing the present invention a rough calculation of the contained oxygen in the iron charge is first obtained and then an excess of carbon (over that stoichiometrically necessary for reaction with the oxygen) is added to the charge. The

furnace is then pumped down to a low total pressure on the order of 0.001 mm. and the charge is heated up to a temperature on the order of about 1650° C. As the charge reaches this high temperature the reaction of carbon and oxygen to form carbon monoxide will proceed at a relatively high rate, causing the pressure in the vacuum system to rise correspondingly, depending upon the pumping capacity of the system. As the rate of carbon monoxide evolution falls, due to the deoxidation of the iron, the pressure in the system also falls. However, the pressure, in itself, is not a reliable measure of the carbon monoxide evolution rate or of the carbon and oxygen balance in solution which corresponds to a given carbon monoxide evolution rate. This is due to the fact that the pressure is affected by the design and condition of the pumping system, by the weight of metal in the charge, by the contamination of the system, and by numerous other variables which cannot be adequately compensated for in commercial practice. It is, therefore, not significant to state that the attainment of a pressure of ten microns, for example, is indicative of a certain carbon and oxygen balance in the melt from one day to the next, or even from one melt to the next. Furthermore, while the carbon and oxygen contents are still relatively high, the oxygen content serves as a limitation on both the equilibrium and kinetics of the reaction of iron with magnesium, and the carbon reacts rapidly with any added oxygen from the crucible reaction. However, when the carbon and oxygen in solution get quite low, there comes a point beyond which the carbon has reduced the oxygen in solution to so low a value that diffusion in the boundary layer next to the crucible, and subsequent distribution of oxygen by molten currents, becomes more dominant than the deoxidation effect of the carbon. The oxygen content of the melt then begins to rise in a relatively rapid approach toward the equilibrium which exists between the molten iron and the crucible material.

This general behavior can be well illustrated in Fig. 1 in which carbon, oxygen, nitrogen, and hydrogen contents are plotted as a function of time during which a charge of iron was held at a relatively constant temperature of about 1650° C. From this Fig. 1 it may be seen that while the carbon content decreases rapidly, the oxygen content also decreases rapidly. However, at a certain time a minimum in oxygen content is obtained. Beyond this time the oxygen content begins to increase quite rapidly. Meanwhile, the nitrogen and hydrogen contents have fallen to very low values.

It has been found that the approach to this minimum oxygen content, illustrated in Fig. 1, is marked by a rapid decrease in the rate of evolution of carbon monoxide. Furthermore, when the melting practice is standardized with respect to the amount of carbon added to insure an excess over the oxygen content, and the temperature is controlled closely, the rate of carbon monoxide evolution, at which the minimum oxygen content is reached, is relatively constant. If the evolution rate is measured at short time intervals, as more fully described hereinafter, this critical rate may be readily detected and the reaction between the crucible and the molten charge may be arrested. This arresting of the reaction may be achieved in several ways. In one way the charge may be poured from the crucible into a suitable mold. In another, the vacuum furnace may be flooded with a relatively high pressure (such as an atmospheric pressure) of an inert gas such as argon, helium, or the like. This atmospheric pressure of the argon will suppress the iron-magnesia reaction.

Referring now to Fig. 2 there is shown a curve wherein the weight percentage of oxygen in the iron is plotted against the carbon monoxide evolution rate in micron cubic feet per minute per pound of iron. When the carbon monoxide evolution rate is above 40 micron cubic feet per minute per pound of iron, the weight of contained oxygen can be very substantial. However, as the

carbon monoxide evolution rate falls to about 20, the oxygen content in the iron has fallen drastically to below .02. From this point the carbon monoxide evolution rate continues to fall, as does the oxygen content of the iron, until a carbon monoxide evolution rate of about 4 micron cubic feet per minute per pound of iron is reached. At this point the carbon has been almost entirely used up and the equilibrium reaction between the iron and the crucible begins to be the controlling factor in the oxygen content, and as the carbon monoxide evolution rate decreases further the oxygen content drastically increases. As a consequence, in the practice of the present invention the iron is poured, or the crucible reaction is otherwise stopped (such as by flooding with argon) after the time when the carbon monoxide evolution rate has dropped to below about 20 micron cubic feet per minute per pound and before the time when the carbon monoxide evolution rate has fallen to about 4 micron cubic feet per minute per pound.

In a preferred embodiment of the invention this critical evolution rate is set between about 18 and 8 micron cubic feet per minute per pound of iron. This is due to the fact that it is desired to assure oxygen contents of less than about .015% as a higher limit. The lower limit is set by the fact that there is an appreciable time lag during the determination of the carbon monoxide evolution rate. If it is attempted to reach the absolute minimum carbon monoxide evolution rate, it is quite possible that the crucible reaction may be the controlling factor because of the time that the carbon monoxide rate determination requires.

In one specific embodiment of the invention the following procedure is followed.

#### Example I

A charge of iron, in the form of 30 lbs. of carbonyl "L" iron stock, is added to a magnesia crucible. To this iron charge there is added approximately 12 grams of carbon in either massive or powder form, but preferably the former. The furnace containing the crucible is then evacuated to a low free air pressure on the order of .001-.010 mm. Hg abs. When this low pressure is obtained the iron charge in the crucible is heated as rapidly as possible, such as by the use of an induction coil, to a preferred refining temperature on the order of about 1650° C. As a result of this heating a pressure rise is caused by the very rapid evolution of carbon monoxide. When the temperature has leveled off at about 1650° C., carbon monoxide evolution rates are determined about every five minutes. This reading may be readily obtained by valving off the pumping system and measuring the pressure rise. This pressure rise is directly related to the carbon monoxide evolution rate (E) and can be calculated from the following formula:

$$E = \frac{nV}{W}$$

where *n* is the pressure rise in microns Hg abs. per minute, *V* is the effective volume of the vacuum system in cubic feet, and *W* is the weight of the iron charge in pounds.

When the evolution rate (E) has fallen to less than about 20 micron cubic feet per minute per pound of iron, preferably less than about 18 micron cubic feet per minute per pound of iron, the charge may be poured into a suitable mold therefor if pure iron is to be made. If an alloy is to be made the vacuum furnace may be flooded with an atmosphere of inert gas when the critical carbon monoxide evolution rate has been reached.

#### Example II

The operating procedures are identical to those described in Example I except that, after initially pumping down the system to a low free air pressure on the order of .001-.010 mm. Hg abs., an inert gas pressure on the order of 100 mm. Hg abs. is introduced into the system

prior to the melting of the charge. This has the effect of preventing the carbon-oxygen reaction until the melt has been brought up to the desired temperature. When this desired temperature, such as 1600° C. or above, has been reached, the inert gas pressure is pumped out of the system and the carbon-oxygen reaction is allowed to proceed.

*Example III*

The same techniques are employed as in Example I. However, when the critical low carbon monoxide evolution rate has been reached an inert gas pressure of between 50 mm. and 760 mm. Hg<sub>abs</sub> of argon is introduced into the vacuum furnace. There are then added to the molten iron the additions necessary to give a final steel composition within the following composition range based on the weight of the iron charge:

0.95-1.10 wt. percent carbon  
0.25-0.45 wt. percent manganese  
0.005 wt. percent maximum phosphorus or sulfur  
0.20-0.35 wt. percent silicon  
1.30-1.60 wt. percent chromium  
Balance iron

This charge is then stirred, such as by use of induced currents, until the addition elements are thoroughly mixed into the melt. This stirring may be continued for about 5-10 minutes. This procedure will give a steel which corresponds closely with S. A. E. 52100 Steel. By practicing the present invention such a steel has been found to have oxygen and nitrogen contents on the order of 0.005% and 0.0005%, respectively. Such a steel having this low gas content, either dissolved or in the form of inclusions, has been found to have superior fatigue strength characteristics for application in bearings and the like. By the use of this invention, the quantities of the other alloying elements, such as carbon, can be maintained within much narrower ranges than those normally specified for such alloys so as to provide more uniform response to heat treatment and a smaller spread in physical properties.

While the principles of the invention have been described specifically above in connection with the preferred embodiments thereof, it would seem advisable to point out, in more detail, the critical dynamic relationship of the invention as distinguished from the static purification systems of the prior art discussed earlier in the specification. For this purpose reference should be had to Fig. 3 wherein four curves of total oxygen content in molten iron are plotted against total pressure in microns. Of these curves, curve A shows a system where there is a maximum pumping capacity (i. e., there is a large, high-vacuum pump which is operating at full capacity with a clean vacuum system which is not outgassing). As can be seen from curve A, the minimum oxygen content occurs at a low total pressure of less than about 1.5 microns. Curve B illustrates the situation when the pumping capacity is somewhat decreased, for example due to deteriorated pump oil. In curve B the minimum oxygen content corresponds to a total pressure of approximately 12 microns. With curve C, which represents an even lower pumping capacity, the minimum oxygen content occurs at approximately 20 microns, while the oxygen content at a pressure of 1½ microns is on the order of about 1%, or the equilibrium between the iron and the magnesia crucible. The same situation is true with respect to curve D which represents a minimum pumping capacity.

From an examination of the curves in Fig. 3 it should be readily apparent that static determination of the oxygen content as a function of total pressure in the vacuum furnace is completely useless unless it is known exactly which curve is actually being utilized during the pump-down. As explained previously, variations in the size of the melt in addition to the humidity of the atmosphere, cleanliness of the interior of the vacuum furnace, cleanli-

ness of the pump oil, and numerous other variables make it enormously difficult to predict the pumping capacity of the system at any given time. However, it is quite simple to measure the carbon monoxide evolution rate and to utilize this dynamic standard as the control for determining oxygen content.

Referring now to Fig. 4 there is shown a diagrammatic illustration of a vacuum furnace pumping system, and related control elements, arranged for practicing the present invention. In this Fig. 4 the vacuum furnace is indicated at 10 and has associated therewith a suitable pumping system 12. This pumping system may be of the type normally utilized in vacuum metallurgy, and may include a diffusion pump in combination with a mechanical vacuum pump. Between the furnace 10 and the pumping system 12 there is situated a valve 14 which can be operated to isolate the vacuum furnace from the pumping system. The pressure in the vacuum furnace is arranged to be read by an "Alphatron" 16 of the type disclosed in U. S. Patent No. 2,497,213. Other suitable pressure gauges may equally be employed.

Valve 14 is arranged to be closed by a timer circuit 18, this timer circuit being closed by a valve-closing and timer-starting circuit 20 which can be automatically or manually operated at predetermined periods of time to isolate the vacuum furnace from the pumping system and to measure the time during which this isolation is accomplished. The output signal from the "Alphatron" pressure gauge 16 is fed to an indicating needle 22, the position of which, with respect to a rotatable scale 23, is controlled by the pressure in the vacuum furnace 10 as read by the "Alphatron" 16. Carried by the rotatable scale 23 is a segmental element 24 which, when contacted by the needle 22, is arranged to close a contact circuit 30. The needle 22 is arranged so that it will normally pass over the segmental contact 24 without engaging this contact 24. However, when solenoid 26 is operated by the timer circuit 18, the needle is pressed downwardly against the dial 23. If the needle 22 should be over the contact element 24, the contact circuit 30 will be closed. The rotatable scale 23 is preferably also suitably graduated so that it will read directly the carbon monoxide evolution rate in micron cubic feet per minute per pound of iron being melted in the vacuum furnace 10.

The contact circuit 30 is preferably arranged so as to actuate an arresting mechanism 32 associated with the vacuum furnace or a signal which will indicate to the furnace operator that a predetermined carbon monoxide evolution rate has been obtained. The control circuit also includes, in a preferred embodiment, an automatic zero set mechanism 34 which will align the "0" on the scale 28 with the needle 22 at the beginning of the timing circuit. This alignment can, of course, be made manually at the time the timing cycle is commenced.

Referring now to the operation of Fig. 4, when it is desired to measure the carbon monoxide evolution rate in the furnace, the operator actuates the valve closing and timing starter circuit 20. This immediately actuates the zero set mechanism 34 so that, at zero time, the "0" indication on the scale 28 is positioned under the needle 22. The timer circuit 18 also is started, this timer circuit closing the valve 14. The vacuum furnace 10 is now isolated from the pumping system, and the pressure therein begins to rise due to carbon monoxide evolution. This pressure rise is read by the "Alphatron" 16, thus causing the needle 22 to move to the right across the face of the scale 23. If the carbon monoxide evolution rate is high the needle 22 will move rapidly. When the solenoid 26 is actuated at the end of a predetermined time which, for convenience, may be one minute, it will press the needle 22 against the rotatable scale 23. Since the needle has been moving rapidly, it will have passed the contact element 24 and the contact circuit 30 will not be energized. Valve 14 is then opened, either automatically or manually, and the vacuum pumping system is used to

again reduce the pressure in the furnace. Another reading is taken at an interval of about five minutes, either automatically or manually, and the measuring cycle is repeated. The operation is repeated until such time as the carbon monoxide evolution rate has dropped below about 20 micron cubic feet per minute per pound of iron. When this low carbon monoxide evolution rate has been achieved, the movement of the needle 22, with respect to the rotatable scale 23, will be relatively slow. Thus, when the solenoid 26 is energized to indicate the end of the measuring cycle, the needle 22 will be pressed against the contact element 24 and the contact circuit will be closed. This will energize either the signal system or the arresting mechanism depending upon whether or not the system is completely automatic. When the signal circuit has been energized, the operator may decide to continue to pump down the system if the needle indicates that the carbon monoxide evolution rate is still around 18 micron cubic feet per minute, and may take another reading a few minutes later so as to strike the lowest possible point on the oxygen curve. When the desired carbon monoxide evolution rate has been obtained, the operator may flood the tank with argon, if desired, or may pour the charge from the crucible into a suitable mold therefor. Alternatively, he may adjust the contact element 24 to energize the arresting mechanism at a lower evolution rate than 20 micron cubic feet per minute per pound. The arresting mechanism may be either a gas flooding system or a pouring mechanism, the former being preferred when alloys are to be made.

Numerous other control circuits may be employed in lieu of the one specifically illustrated, and numerous other pressure measuring techniques may be utilized. While direct indicating and direct reading instruments are naturally preferred, other techniques for determining the carbon monoxide evolution rate in any instant of time can be substituted without departing from the spirit of the invention.

When additions are to be made to the molten iron charge, it is preferred that a furnace of the type shown in my copending application Serial No. 187,016, filed September 27, 1950, now U. S. Patent No. 2,625,719, be employed. This furnace has the additional advantage that the next charge of iron may be added to the furnace without opening the furnace interior to the atmosphere and thus any residual iron in the crucible is kept free of air oxidation.

Since certain changes may be made in the above product, process, and apparatus without departing from the scope of the invention herein involved, it is intended that all matter contained in the above description, or shown in the accompanying drawing, shall be interpreted as illustrative and not in a limiting sense.

What is claimed is:

1. The process of manufacturing high purity iron and alloys of iron having an oxygen content by weight of less than about 0.015% and a carbon content by weight of less than about 0.005%, said process comprising the steps of confining said iron in a vacuum furnace in a crucible predominating in an oxide of a metal having a high vapor pressure at the temperature of molten iron, adding to said iron, at some stage in said process, an amount of carbon in excess of the amount needed for stoichiometrically reacting with the oxygen in said iron, evacuating said furnace, heating said iron and carbon to a temperature on the order of about 1650° C., maintaining said temperature substantially constant, measuring the rate of evolution of carbon monoxide from said molten iron resulting from reduction of iron oxide by said added carbon, and pouring said iron into a mold between the time when the carbon monoxide evolution rate falls to about 20 micron cubic feet per minute per pound of iron and before the carbon monoxide evolution rate falls to about 4 micron cubic feet per minute per pound of iron.

2. The process of manufacturing high purity iron and

alloys of iron having an oxygen content by weight of less than about 0.015%, said process comprising the steps of confining said iron in a vacuum furnace in a crucible predominating in an oxide of a metal having a high vapor pressure at the temperature of molten iron, adding to said iron, at some stage in said process, an amount of carbon in excess of the amount needed for stoichiometrically reacting with the oxygen in said iron, evacuating said furnace, heating said iron and carbon to a temperature on the order of about 1650° C., maintaining said temperature substantially constant, measuring the rate of evolution of carbon monoxide from said molten iron resulting from reduction of iron oxide by said added carbon, and arresting the reaction between the molten iron and the crucible at some point between the time when the carbon monoxide evolution rate falls to about 20 micron cubic feet per minute per pound of iron and before the carbon monoxide evolution rate falls to about 4 micron cubic feet per minute per pound of iron.

3. The process of manufacturing a high purity iron alloy having an oxygen content by weight of less than about 0.015%, said process comprising the steps of confining said iron in a vacuum furnace in a crucible predominating in an oxide of a metal having a high vapor pressure at the temperature of molten iron, adding to said iron, at some stage in said process, an amount of carbon in excess of the amount needed for stoichiometrically reacting with the oxygen in said iron, evacuating said furnace, heating said iron and carbon to a temperature on the order of about 1650° C., maintaining said temperature substantially constant, measuring the rate of evolution of carbon monoxide from said molten iron resulting from reduction of iron oxide by said added carbon, arresting the reaction between the molten iron and the crucible at some point between the time when the carbon monoxide evolution rate falls to about 20 micron cubic feet per minute per pound of iron and before the carbon monoxide evolution rate falls to about 4 micron cubic feet per minute per pound of iron, and adding at least one alloying element to said deoxidized iron to form a high purity iron alloy.

4. The process of purifying iron to obtain a molten iron containing, by weight, less than about .005% carbon and less than about .015% oxygen, said process comprising the steps of confining said iron in a vacuum furnace in a crucible predominating in an oxide of magnesium, adding to said iron at some stage in said process, an amount of carbon in excess of the amount needed for stoichiometrically reacting with the oxygen in said iron, evacuating said furnace, heating said iron and carbon to a temperature on the order of about 1650° C., maintaining said temperature substantially constant, measuring the rate of evolution of carbon monoxide from said molten iron resulting from reduction of iron oxide by said added carbon, and arresting the reaction between the molten iron and the crucible at some point between the time when the carbon monoxide evolution rate falls to about 20 micron cubic feet per minute per pound of iron and before the carbon monoxide evolution rate falls below about 4 micron cubic feet per minute per pound of iron.

5. The process of purifying iron to obtain a molten iron containing, by weight, less than about .005% carbon and less than about .015% oxygen, said process comprising the steps of confining said iron in a vacuum furnace in a crucible predominating in an oxide of magnesium, adding to said iron at some stage in said process, an amount of carbon between about 25% and 50% in excess of the amount needed for stoichiometrically reacting with the oxygen in said iron, evacuating said furnace, heating said iron and carbon to a temperature on the order of about 1650° C., maintaining said temperature substantially constant, measuring the rate of evolution of carbon monoxide from said molten iron resulting from reduction of iron oxide by said added carbon, and ar-

resting the reaction between the molten iron and the crucible at some point between the time when the carbon monoxide evolution rate falls to about 18 micron cubic feet per minute per pound of iron and before the carbon monoxide evolution rate falls below about 8 micron cubic feet per minute per pound of iron. 5

6. The process of claim 2 wherein the reaction between the molten iron and the crucible is arrested by creating in said vacuum furnace an atmosphere of an inert gas having a total pressure in excess of 50 mm. 10 Hg abs.

7. The process of claim 6 wherein at least one alloying constituent is added to said molten iron after said inert gas is introduced into said furnace chamber.

8. The process of claim 2 wherein the reaction between the molten iron and the crucible is arrested by pouring said molten iron out of said crucible. 15

## References Cited in the file of this patent

## UNITED STATES PATENTS

|           |                  |                |
|-----------|------------------|----------------|
| 1,555,314 | Rohn             | Sept. 29, 1925 |
| 2,036,496 | Randolph         | Apr. 7, 1936   |
| 2,054,922 | Betterton et al. | Sept. 22, 1936 |
| 2,071,942 | Rohn             | Feb. 23, 1937  |
| 2,076,800 | Thummel          | Apr. 13, 1937  |
| 2,155,349 | Mathesius et al. | Apr. 18, 1939  |
| 2,513,935 | Harris           | July 4, 1950   |
| 2,587,793 | Waldron          | Mar. 4, 1952   |

## FOREIGN PATENTS

|        |        |               |
|--------|--------|---------------|
| 40,649 | Norway | Dec. 22, 1924 |
|--------|--------|---------------|

## OTHER REFERENCES

Yensen, volume XXXII, Transactions of the American Electrochemical Soc. (1917), pages 178 and 179.